

## [54] PHOSPHATE ROCK FLOTATION

[75] Inventor: David Lawrence Johnston,  
Yellowknife, Canada[73] Assignee: Cominco Ltd., Montreal, Quebec,  
Canada

[22] Filed: Dec. 13, 1971

[21] Appl. No.: 207,099

[52] U.S. Cl. 209/166

[51] Int. Cl. B03d 1/02

[58] Field of Search 209/166

## [56] References Cited

## UNITED STATES PATENTS

|           |         |        |           |
|-----------|---------|--------|-----------|
| 1,914,695 | 6/1933  | Lange  | 207/166   |
| 2,553,905 | 5/1951  | Evans  | 209/166 X |
| 2,303,931 | 12/1942 | Greene | 209/166   |
| 2,698,088 | 12/1954 | Pryor  | 209/166   |

|           |         |         |           |
|-----------|---------|---------|-----------|
| 3,113,838 | 12/1963 | Perri   | 209/166 X |
| 3,405,802 | 10/1968 | Prellen | 209/166   |
| 3,462,016 | 8/1969  | Bushell | 209/166   |
| 3,462,017 | 8/1969  | Bushell | 209/166   |

Primary Examiner—Robert Halper

## [57] ABSTRACT

A process for beneficiating phosphate rock containing siliceous and carbonaceous gangue materials and gypsum which comprises the steps of subjecting comminuted phosphate rock to a first stage anionic flotation step to float phosphates from siliceous material, conditioning the float product in an aqueous solution containing added phosphate ion and sulphate ion, subjecting the conditioned float product to a second stage anionic flotation step and recovering a concentrate product of high phosphate-bearing mineral content.

5 Claims, 1 Drawing Figure



PATENTED APR 30 1974

3,807,556



INVENTOR.  
DAVID L. JOHNSTON

BY

*Anne J. Fors*

Agent

## PHOSPHATE ROCK FLOTATION

## BACKGROUND OF THE INVENTION

This invention relates to a process for beneficiating phosphate bearing materials and is particularly directed to a flotation process for the concentration of phosphate minerals in phosphate rock high in silica, calcium carbonate, magnesium carbonate and gypsum.

U.S. Pat. Nos. 3,462,016 and 3,462,017 describe processes for the beneficiation of phosphate-bearing materials high in silica and in carbonates such as calcium carbonate and magnesium carbonate. The former patent teaches a two-stage anionic flotation process in which the bulk of the silica is removed as an underflow and the phosphate minerals and carbonates are removed as float in the first stage, and the phosphate minerals selectively depressed for removal as an underflow concentrate and the calcium and magnesium carbonates floated in the second stage; the float from the first stage being conditioned by the addition of phosphoric acid for depression of the phosphate minerals in the second stage. The latter patent teaches a two-stage anionic process wherein the phosphate minerals are selectively depressed prior to the second stage flotation by the addition of a soluble alkali phosphate to the flotation circuit.

## SUMMARY OF THE INVENTION

Although the processes taught in the aforesaid patents are effective for the beneficiation of phosphate-bearing materials high in silica and in carbonates, it has been found that undesirable phosphate losses occur from the flotation solutions in the presence of gypsum. I have found surprisingly that the presence of a sulphate ion such as produced by a soluble sulphate salt, added in addition to the alkali phosphate or phosphoric acid in the conditioning step, results in a substantial reduction in the loss of soluble phosphate with significant economies in the operation of the process in that the cost of the sulphate salt consumed is considerably less than that of the additional phosphate recovered.

It is a principal object of the present invention therefore to provide an improved process for the beneficiation of phosphate-bearing materials containing gypsum for the recovery of phosphate minerals with minimum phosphate losses.

## BRIEF DESCRIPTION OF THE DRAWING

This and other objects of the process of the invention and the manner in which they can be attained will become apparent from the following detailed description of the process taken in conjunction with the drawing, in which:

The FIGURE illustrates by graph the effect of the presence of soluble sulphate on the quantity of phosphate ions in solution.

## DESCRIPTION OF THE PREFERRED EMBODIMENT

As described in the above-noted patents, the  $H_2PO_4^-$  ions provided through the addition of phosphoric acid or alkali phosphate in the conditioning step effectively deactivate the residual anionic collector on the surfaces of the phosphate particles while not affecting the activated surfaces of the calcium carbonate and mag-

nesium carbonate particles. Thus, in the succeeding second stage anionic flotation an improved separation of calcium carbonate and magnesium carbonate from the phosphate minerals is achieved.

Although it will be understood that I am not bound by hypothetical considerations, it is believed that any gypsum contained in the ore causes a loss of soluble phosphate from the solution through reaction of orthophosphate ions with gypsum for precipitation of a brushite ( $CaHPO_4 \cdot 2H_2O$ ) surface layer or coating on the gypsum. A sufficient quantity of soluble phosphate must of necessity be added in the conditioning step, therefore, over and above that which becomes precipitated out by gypsum, in order to effectively accomplish the de-activation of the anionic collector on the surfaces of the phosphate particles. By means of the present process, the loss of soluble phosphate, such as ammonium phosphate, from the solution can be avoided or greatly reduced. This is of economic significance to the process for the phosphate make-up requirements are reduced to quantities necessary to compensate for physical losses only. The actual quantity saved will vary with the gypsum content of the first stage concentrate and may range from 5 to 20 lbs/ton equivalent of the final concentrate. Furthermore, it has been found that the presence of sulphate ions in the pulp does not adversely affect the flotation results.

The explanation in simple terms for loss of soluble phosphate because of the gypsum in ore is found in the equation:



This reaction can be hindered or prevented by adding soluble sulphates.

Another important reaction taking place in the system is:



which, in conjunction with reaction (1) being held to the left in the presence of an adequate concentration of sulphate ions, can lead to a release of phosphate from the ore to solution. It may be seen then that an optimum addition of soluble sulphate to the process is of some importance, for an excess addition will result in minor losses to solution of the phosphate it is being attempted to recover from the ore.

I have found that, of the major mineral components present in the phosphate flotation system, gypsum is the only mineral to remove significant quantities of orthophosphate ions from solution and the presence of from about 3 to about 6 g/l, preferably about 4 g/l, of  $Na_2SO_4$  or the presence of from about 2 to about 6 g/l, preferably about 3 g/l  $(NH_4)_2SO_4$ , effectively suppresses the reaction between gypsum and orthophosphate ions, as shown in the FIGURE.

The concentration of orthophosphate ion necessary to depress apatite in the flotation of ores could be decreased by supplying sulphate ion to reduce  $HPO_4^{2-}$  ion loss through  $CaHPO_4 \cdot 2H_2O$  formation. The sulphates useful in the two-stage re flotation process must have the effect of increasing the concentration of sulphate ion in the solutions and the only useful sulphates

are those soluble sulphates which are in a salt form such as sodium, potassium and ammonium sulphates. Sulphuric acid is not satisfactory for this purpose in that the materials on which the two-stage anionic processes are practiced contain calcite and dolomite and the well-known reaction of sulphuric acid with calcite and dolomite produces the undesirable reaction products of gypsum, magnesium sulphate and carbon dioxide. The reactions are rapid and will continue as long as sulphuric acid is added or calcite and dolomite remain. The effect of adding sulphuric acid thus does not include raising the sulphate ion concentration in solution above the gypsum saturation level and sulphuric acid would therefore complicate the gypsum exchange of sulphate for soluble phosphate by introducing more gypsum.

The following example shows the effectiveness of the addition of a soluble sulphate salt to the conditioning step in the process of treating collophane phosphate rock of the type treated according to the processes of the above noted patents. A first stage flotation concentrate was prepared and aliquots of this concentration, containing 0.1 percent sulphate sulphur corresponding to about 0.5 percent gypsum content, were treated by phosphate pulp reflootation for removal of calcite and dolomite, as described in the aforesaid patents. The following amounts of soluble sulphate were added to the flotation solution which contained 10 g/l  $\text{NH}_4\text{H}_2\text{PO}_4$ :

| Test 1 | Sulphate                     | Amount | Remarks                                  |
|--------|------------------------------|--------|------------------------------------------|
| 2      | $\text{Na}_2\text{SO}_4$     | 3 gpl  | Nil Standard $\text{P}_2\text{O}_5$ loss |
| 3      | $\text{Na}_2\text{SO}_4$     | 15 gpl | Reduced loss of $\text{P}_2\text{O}_5$   |
| 4      | $(\text{NH}_4)_2\text{SO}_4$ | 10 gpl | Gain of $\text{P}_2\text{O}_5$           |

Losses of soluble phosphate were determined by measuring and assaying all filtrates and wash waters, with the following results:

- Test 1—11.8 lb/ton  $\text{P}_2\text{O}_5$  loss from solution
- Test 2—1.1 lb/ton  $\text{P}_2\text{O}_5$  loss from solution
- Test 3—2.0 lb/ton  $\text{P}_2\text{O}_5$  gain to solution

Test 4—4.6 lb/ton  $\text{P}_2\text{O}_5$  gain to solution

It will be evident from the foregoing test results illustrated graphically in the FIGURE that, for a gypsum content of at least 0.5 percent in the first stage concentrate, the optimum sulphate addition would be from about 3 to about 6 g/l, preferably about 4 g/l, for  $\text{Na}_2\text{SO}_4$  and would be about 2 to about 6 g/l, preferably about 3 g/l, for  $(\text{NH}_4)_2\text{SO}_4$ .

What we claim as new and desire to protect by letters 10 patent of the United States is:

1. In a process for beneficiating phosphate rock containing siliceous and carbonaceous gangue materials and gypsum in which soluble phosphates are lost by association with the gypsum and which includes the steps 15 of subjecting comminuted phosphate rock to a first stage anionic flotation step for depressing siliceous material, conditioning the float product in an aqueous solution containing added phosphate ion, subjecting the conditioned float product to a second stage anionic flotation step and recovering a concentrate product of high phosphate-bearing mineral content, the improvement which comprises adding a soluble sulphate salt selected from the group consisting of sodium sulphate and ammonium sulphate to the aqueous solution in said conditioning step whereby the losses of phosphates are reduced.
2. In a process as claimed in claim 1, adding from about 3 to about 6 g/l of  $\text{Na}_2\text{SO}_4$  to the aqueous solution in the conditioning step.
3. In a process as claimed in claim 1, adding about 4 g/l of  $\text{Na}_2\text{SO}_4$  to the aqueous solution in the conditioning step.
4. In a process as claimed in claim 1, adding from about 2 to about 6 g/l of  $(\text{NH}_4)_2\text{SO}_4$  to the aqueous solution in the conditioning step.
5. In a process as claimed in claim 1, adding about 3 g/l of  $(\text{NH}_4)_2\text{SO}_4$  to the aqueous solution in the conditioning step.

\* \* \* \* \*

40

45

50

55

60

65